

## UNITED STATES PATENT OFFICE

2,359,782

## BLEACHING PROCESS AND COMPOSITION

Ralph R. Oliver, Lockport, N. Y., assignor to  
Lockport Cotton Batting Co., Lockport, N. Y.No Drawing. Application March 31, 1941,  
Serial No. 386,083

14 Claims. (CL 252—187)

This invention relates to the bleaching of cellulose fibers, such as exist in cotton textiles and in cotton and wood pulp for example. Heretofore, halogen containing, bleaching agents, such as sodium and calcium hypochlorites, for example, have been employed extensively in solutions to bleach cellulose fibers, but results have not been entirely satisfactory due to the adherence to, or deposit upon, the cellulose fibers of encrusting materials during the bleaching process. Such deposits are objectionable because they weaken or embrittle the bleached fibers and destroy or conceal the natural luster and brilliance of the fibers.

I have discovered that the bleaching of cellulose fibers in any form may be hastened or accelerated and a bleached product of better quality obtained by performing the bleaching action with a halogen containing, bleaching agent in the presence of an inorganic glucosate which may be coagulated by bi-valent ions so as to form colloidal particles around the encrusting mineral matter. These glucosates are preferably the inorganic salts or compounds of beta glucoside and its derivatives by condensation reactions. Examples of such glucosates which I have found very satisfactory for this purpose and which are typical of materials of this type are sodium-glucosate, phospho-glucosate, pyro-glucosate and tetra-phospho-glucosate. Glucosates of this type may be coagulated by bi-valent ions and apparently form colloidal particles or insoluble hydrophilic gels around the encrusting mineral and other foreign matter and hold the scale or encrustation forming elements in what may be aptly termed delayed precipitation during the bleaching process. Thus, the glucosates convert the materials in the bleaching solution and on the fibers which would normally tend to form an encrustation on the fibers, into nonadherent suspensoids which hold the encrusting materials in the form of suspended colloids and remain in suspension in the liquid bleaching bath. After the bleaching action, the colloids may be separated from the cellulose fibers by draining off the bath with the suspended colloids and washing the fibers.

The scale or encrustation forming products commonly encountered in a bleaching bath are calcium, magnesium, silicon, iron, carbonates, sulphates and organic materials such as oils, fats, waxes and living organisms. While the exact action of these inorganic beta glucosates in inhibiting the deposits of encrusting materials upon the fibers is not definitely known, it is believed

that their action may be regarded as a state and not a form of matter, and that the action is apparently physical as well as chemical.

In the manufacture of so called chemical cotton and chemical cellulose from wood pulp where a low ash is of prime importance, this improved process is particularly advantageous because an analysis of pulp bleached by this improved process shows a decrease of from sixteen to thirty-three percent less ash, apparently through the prevention of the adherence of encrusting materials to the bleached fibers. I have also found that cellulose fibers of any kind which are bleached in the presence of the inorganic beta glucosates have a better luster and greater brilliancy than can be obtained by the bleaching processes heretofore employed, apparently because they are free from encrusting chemicals or materials. Equally satisfactory results are obtained in the bleaching of chemical wood pulp obtained by the soda process, the sulphate process and modifications of the sulphate process known as the Kraft process where the manufacture of a strong paper sheet is required. The fibers bleached by this improved method have greater strength than has heretofore been possible, because they are not embrittled by any encrusting scale or chemicals, and hence this process is also particularly useful for the bleaching of cotton that is to be fabricated by carding and garnetting, where fiber strength is important. I have also discovered that these same inorganic beta glucosates apparently act as catalysts on the bleaching action and by speeding up the bleaching reaction, the time required for a bleaching action is materially decreased.

The proportions of the glucosate to be employed may be varied to some extent, depending upon the character of the fibers and of the encrusting materials that may be present, as determined by ionic analysis. Generally, excellent results may be obtained by using from one to one hundred parts by weight of the glucosate per million parts of the hypochlorite bleaching solution, but ordinarily, it is unnecessary to use more than twenty-five parts of glucosate per million parts of bleaching solution. It is believed that the glucosides and glucosates which have been mentioned are sufficiently identified by these names, but as a matter of record, and by way of example, the beta glucosides from which satisfactory inorganic glucosates may be formed may be represented by the following formula in which R is a hydrocar-

bon radical depending upon the material from which the glucoside is formed:

Beta glucoside



Glucosates formed from such a glucoside and which are excellent catalysts and inhibiting materials in the present process are:

Sodium-glucosate



Phospho-glucosate



Pyro-glucosate



Tetra-phospho-glucosate



In order to further explain the nature of my discovery, reference may be had to the following specific examples in which the discovery is given practical application:

Example A

50 grams of caustic boiled and washed cotton linters treated for three hours with 400 ml. of cold calcium hypochlorite containing 6 grams per litre of active chlorine.

After bleaching the stock was washed free from active chlorine and dried to bone dry base.

The stock bleached to a brightness of 70 G. E. (The brightness of a standard magnesia block being 100 G. E.)

Ash contents—0.75%.

Example B

50 grams of the same caustic boiled and washed cotton linters treated for three hours with 400 ml. of cold calcium hypochlorite containing 6 grams per litre of active chlorine and entrained in this solution 25 P. P. M. (parts per million) of tetra-phospho-glucosate.

After bleaching, the stock was washed free from active chlorine and dried to bone dry base. The stock bleached to a brightness of 75 G. E.

Ash contents—0.63%.

Comparison of Results A and B

Difference in brightness—7%.

Difference in ash—16%.

Example C

50 grams of caustic boiled and washed cotton linters treated for three hours with 400 ml. of cold calcium hypochlorite containing 6 grams per litre of active chlorine.

After bleaching, the stock was washed free from active chlorine and dried to bone dry base.

The stock bleached to a brightness of 70 G. E.

Ash contents—0.73%.

Example D

50 grams of the same caustic boiled and washed cotton linters treated for three hours with 400 ml. of cold calcium hypochlorite containing 6 grams per litre of active chlorine and entrained in this solution 50 P. P. M. (parts per million) of tetra-phospho-glucosate.

After bleaching, the stock was washed free from active chlorine and dried to bone dry base. Stock bleached to a brightness of 75 G. E. Ash contents—0.51%.

Comparison of Results C and D

Difference in brightness—7%.

Difference in ash—30%.

Example E

Procedure as in Example D, with an entrainment of 100 P. P. M. (parts per million) of tetra-phospho-glucosate.

Stock bleached to a brightness of 75 G. E.

Ash contents—0.52%.

Example F

Procedure as in Example D, with an entrainment of 10 P. P. M. (parts per million) of tetra-phospho-glucosate.

Stock bleached to a brightness of 70 G. E.

Ash contents—0.655%.

Comparison of Examples E and F shows the extremes of entrainment of tetra-phospho-glucosate for this particular grade of cotton linters.

The amount to be used will vary with different grades of stock to be bleached.

In each example using tetra-phospho-glucosate the cotton reached a brightness of 70 G. E. in two and one-half hours.

The beta glucosates appear to be irreversible colloids which react with alkali and alkaline earth metals to form insoluble hydrophilic gels.

It will be understood that various changes in the details, materials and steps which have been hereinabove described in order to explain the nature of my invention, may be made by those skilled in the art within the principle and scope of the invention, as expressed in the appended claims.

I claim as my invention:

1. An improved method of cold bleaching of cellulose fibers which comprises subjecting the material to be bleached to the action at the same time, of a hypochlorite bleaching agent and a preformed inorganic glucosate of the type which will be coagulated by bi-valent ions to form colloidal particles.

2. An improved method of cold bleaching cellulose fibers in a minimum time interval which comprises subjecting the fibers to a hypochlorite bleaching agent in the presence of a preformed inorganic beta glucosate.

3. An improved method of cold bleaching cellulose fibers in a minimum time interval which comprises subjecting the fibers to a halogen containing, bleaching compound combined with a member of the group consisting of alkali and alkaline earth metals in the presence of a preformed inorganic beta glucosate.

4. An improved method of cold bleaching cellulose fibers which comprises subjecting the fibers to the bleaching action of a hypochlorite bleach in the presence of a preformed inorganic beta glucosate.

5. An improved method of cold bleaching which comprises subjecting the material to be bleached to the action, at the same time, of a hypochlorite bleaching agent and a preformed inorganic glucosate capable of coagulation by bi-valent ions to form colloidal particles and containing an alkali metal.

6. An improved method of cold bleaching of cellulose fibrous materials which comprises subjecting the materials to be bleached to the action

at the same time in a bleaching bath of a hypochlorite, bleaching agent and preformed tetraphospho-glucosate.

7. An improved method of cold bleaching of fibers of vegetable origin which comprises subjecting the fibers to be bleached to a bleaching bath having in solution therein a calcium hypochlorite bleaching agent and preformed tetraphospho-glucosate.

8. The method of cold bleaching of fibers of vegetable origin which comprises subjecting the fibers to be bleached to a bleaching bath, containing a calcium hypochlorite bleaching agent and a preformed inorganic glucosate capable of coagulation by bi-valent ions to form colloidal particles and combined with a salt of phosphoric acid.

9. A bleaching composition operable for the cold bleaching of cellulose fibers in a manner to give the bleached fibers a good luster, a high brilliancy, and freedom from encrusting materials, which comprises a mixture of a hypochlorite bleaching agent and a preformed agent containing an inorganic beta glucosate and capable of coagulation by bi-valent ions to form colloidal particles.

10. A bleaching composition operable for the cold bleaching of cellulose fibers in a manner to give the bleached fibers a good luster, a high brilliancy, and freedom from encrusting materials, which comprises a mixture of a bleaching agent containing a halogen as the bleaching

agent combined with a member of the group consisting of alkali and alkaline earth metals, and a preformed agent containing a glucosate combined with an inorganic salt and capable of coagulation by bi-valent ions to form colloidal particles.

11. A bleaching composition operable for cold bleaching of cellulose fibers comprising a mixture of a hypochlorite bleaching agent with a preformed agent formed of a glucosate combined with an inorganic base containing an alkali metal.

12. A bleaching composition, capable of cold bleaching of cellulose fibers comprising a mixture of a hypochlorite bleaching agent and preformed tetra-phospho-glucosate.

13. A bleaching composition operable for the cold bleaching of cellulose fibers in a manner to give the bleached fibers a good luster, a high brilliancy, and freedom from encrusting materials, which comprises a mixture of a halogen containing bleaching agent combined with a member of the group consisting of alkali and alkaline earth metals and a preformed agent containing tetra-phospho-glucosate.

14. A bleaching composition operable for the cold bleaching of cellulose fibers in a manner to give the bleached fibers a good luster, a high brilliancy, and freedom from encrusting materials, which comprises a mixture of a calcium hypochlorite bleaching agent and a preformed agent containing tetra-phospho-glucosate.

RALPH R. OLIVER.